

## UNITED STATES PATENT OFFICE

1,938,022

## TANNING AGENT

Johann Huismann, Leverkusen-on-the-Rhine, and Gustav Mauthe, Cologne-Holweide, Germany, assignors to I. G. Farbenindustrie Aktiengesellschaft, Frankfort-on-the-Main, Germany

No Drawing. Application February 7, 1931, Serial No. 514,306, and in Germany February 27, 1930

2 Claims. (Cl. 260—129)

The present invention relates to new tanning agents. According to this invention the materials to be tanned in accordance with tanners' practice are treated with a water soluble compound of the general formula:



wherein R stands for an aromatic radical of the benzene, naphthalene or diphenyl series or two similar aromatic radicals of the benzene series which are linked with each other or by means of a bridge, for example, for the grouping  $\text{C}_6\text{H}_5\text{CH}_2-\text{CH}_2-\text{C}_6\text{H}_5$ ,  $\text{C}_6\text{H}_5\text{CH}=\text{CHC}_6\text{H}_5$ ,  $\text{C}_6\text{H}_5-\text{O}-\text{C}_6\text{H}_5$ ,  $\text{C}_6\text{H}_5-\text{NH}-\text{CO}-\text{NH}-\text{C}_6\text{H}_5$ , and  $\text{R}_1$  and  $\text{R}_2$  stand for the same or different sub-

Drenched, unhaired goats' skins (free from lime) are treated with 25% of almost completely neutralized but still acetic acid reacting bis-(1:2-dichlorobenzene - 4 - sulfonyl - 3' - aminobenzene-1'-sulfonyl) - benzidine - m - m' - disulfonic acid with the addition of 3.3% of lactic acid in 300% of water until completely tanned. (All the figures given refer to the weight of the unhaired skins.)

The tanning agent is obtainable by condensing bis-(3 - amino - benzene - sulfonyl) - benzidine-m-m' - disulfonic acid (compare British Letters Patent No. 333,559, Example 6) with 1,2-dichlorobenzene-4-sulfochloride analogously to the process as described in Example 5 of the said Letters Patent and corresponds to the formula:



stituted or unsubstituted bi- or polynuclear arylsulfone-arylamide derivatives of the benzene or naphthalene series with chain-like linkage in which the sulfone imide groups combining the aryl nuclei may be partly replaced by aliphatic or aromatic carboxylic acid amide groups, at least one of the nuclei containing a sulfonic acid group. These new tanning agents are generally colorless powders being easily soluble in water. They are obtainable according to methods described in the British Letters Patent No. 333,559, Examples 5 to 7.

The following examples illustrate the invention but without limiting it thereto:

According to the thickness of the skins the tanning requires three to five days. After tanning the skins are well rinsed and oiled from the grain. The finished curried leather is soft, plump and long fibered and shows great similarity to leather tanned with vegetable tanning agents. It differs, however, advantageously from the latter in its pure white color and practically complete fastness to light.

## Example 2

Unhaired skins pickled with a pickle consisting of:—1% of commercial formic acid, 8% of sodium chloride, and 100% of water are tanned in

55

60

65

70

75

80

85

90

95

100

a fulling vessel with 15% strength of partly neutralized bis-(1:2-dichlorobenzene-4-sulfonyl-3'-aminobenzene-1'-sulfonyl)-diamino-stilbene-disulfonic acid of the formula:

This re-tanning confers upon the leather a remarkable fullness. The color of the leather is lighter than that obtained by the often practiced sumach re-tanning.

80

5



having a weakly acid reaction to Congo red in 100% bath without further addition. The bis-(1:2-dichlorobenzene-4-sulfonyl-3'-aminobenzene-1'-sulfonyl)-diamino-stilbene-disulfonic acid may be produced analogously to the process described in Example 1 of British Letters Patent No. 333,559, by causing one molecular proportion of 4,4'-diamino-stilbene-disulfonic acid to react with two molecular proportions of 3-nitro-benzene-sulfochloride, reduction of the resulting condensation product and condensation of the di-

85

30



amino compound with two molecular proportions of 1,2-dichlorobenzene-4-sulfochloride. The tanning agent dissolved in a little water is added in three portions in the course of six hours. The tanning is complete after two days. The finished pure white leather is very similar to that of Example 1.

55

#### Example 3

East Indian sheep skin leather is well fulled in the customary manner and rinsed in running water. Re-tanning follows in 150% of water with 10% of the tanning agent of Example 1 and 1.3% of lactic acid. The time of tanning

One-bath chromium calf leather, thoroughly freed from acid, is fulled for one hour in 150% of water (all the quantities are calculated on the shaving weight) containing 3% of the sodium salt of bis-(1:2-dichlorobenzene-4-sulfonyl-3'-aminobenzene-1'-sulfonyl-3''-aminobenzene-1''-sulfonyl)-benzidine-m-m'-disulfonic acid (British Letters Patent No. 333,559, Example 7) of the formula:

95

100

105

#### Example 4

One-bath chromium calf leather, thoroughly freed from acid, is fulled for one hour in 150% of water (all the quantities are calculated on the shaving weight) containing 3% of the sodium salt of bis-(1:2-dichlorobenzene-4-sulfonyl-3'-aminobenzene-1'-sulfonyl-3''-aminobenzene-1''-sulfonyl)-benzidine-m-m'-disulfonic acid (British Letters Patent No. 333,559, Example 7) of the formula:

110

115

120

125

130

135

140

145

150

1.5% of oxalic acid is then added and fulling continued for three quarters of an hour longer. After that the leather is rinsed in running water for half an hour and well stuffed with 3% of sulfonated neat's-foot oil, at 50° C. The chromium leather thus bleached is almost pure white and possesses almost complete fastness to light.

#### Example 5

Degreased sheep skins (free from lime) treated with a pickle consisting of: 0.5% of formic acid, 6% of sodium chloride, and 100% of water are tanned with a synthetic tanning agent of the probable formula:

65



70

amounts to three hours. The quantities specified are calculated on the striking out weight,

which is obtained by the condensation of bis-(3-aminobenzene-sulfonyl)-benzidine-m-m'-disul-

155

fonic acid (compare British Letters Patent No. 333,559, Example 6) with a mixture of 1,2-dichlorobenzene-4-sulfochloride and 1,4-dichlorobenzene-2-sulfochloride. Therefore it consists of 5 a mixture of symmetrically and asymmetrically constructed compounds of the above mentioned formula. 2.5% of this product are used, and 22

In the examples the tanning agents specified can be replaced by other representatives of the compounds denoted by the general formula. Such products are, for example, the sodium salt of bis-(1:4-dichlorobenzene-2-sulfonyl-3'-amino-80 benzene-1'-sulfonyl-benzidine-m-m'-disulfonic acid.

10.



85

15.



90

20.

parts by weight of a technical 30% acetic acid are added for each 100 parts by weight of the tanning agent.

25 After some hours the tanning is performed with the addition of 10% of the tanning agent, 25 parts by weight of 30% acetic acid and 3 parts by weight of 100% formic acid for each 100 parts by weight of the dry ware.

or of bis-(4-chlorobenzene-1-sulfonyl-3'-aminobenzene-1'-sulfonyl)-benzidine-m.m'-disulfonic acid or of bis-(toluene-4-sulfonyl-3'-aminobenzene-1'-sulfonyl)-benzidine-m.m'-disulfonic acid or of bis-(benzenesulfonyl-3'-aminobenzene-1'-sulfonyl)-benzidine-m.m'-disulfonic acid or of bis-(salicylic acid-sulfonyl-3'-aminobenzene-1'-sulfonyl)-benzidine-m.m'-disulfonic acid:

100

30.



105

35.



110

40.



115

45 The acidified concentrated aqueous solution of the tanning agent is added in several portions in the course of one day. Then it is fulled until

or of bis-(naphthalene-1-sulfonyl-3'-aminobenzene-1'-sulfonyl)-benzidine-m.m'-disulfonic acid:

120

50.



125

55.



130

60 completely tanned and after a short rinsing it is carried in the customary manner. The leather thus obtained shows the same excellent properties as mentioned in Example 1.

or of bis-(naphthalene-2-sulfonyl-3'-aminobenzene-1'-sulfonyl)-benzidine-m.m'-disulfonic acid:

135

65.



140

70.



145

75.

or of bis-(benzenesulfonyl-4'-amino-1'-toluene-2'-sulfonyl)-benzidine-m.m'-disulfonic acid:

aminobenzene-1'-sulfonyl-3''-aminobenzene-1'''-sulfonyl)-diaminostilbene-disulfonic acid:



or of bis-(benzenesulfonyl-4'-amino-1'-chlorobenzene-2'-sulfonyl)-benzidine - m.m'-disulfonic acid:



35 or of bis-(benzoic acid-sulfonyl-3'-aminobenzene - 1' - sulfonyl)-1''5''-naphthalenediamino-3'''7'''-disulfonic acid:



60 or of bis-(1,2-dichlorobenzene-4-sulfonyl-3'-aminobenzene - 1' - sulfonyl)-4''-4'''-diaminodibenzyl-2''-2'''-disulfonic acid:

obtainable by condensing one molecular proportion of the sodium salt of bis-(3-aminobenzene-sulfonyl)-benzidine-m.m'-disulfonic acid (com-



75 or of bis - (1:2-dichlorobenzene - 4 - sulfonyl-3' - pare British Letters Patent No. 333,559, Example 150

6) with two molecular proportions of 3-chloro-phenoxy-acetylchloride according to the methods described in the British Letters Patent 313,110, or of bis-(benzoyl-3'-aminobenzene-1'-sulfonyl)-benzidine-m-m'-disulfonic acid:



obtainable by condensing one molecular proportion of bis-(3-aminobenzene-sulfonyl)-benzidine-m-m'-disulfonic acid (compare British Letters Patent 333,559, Example 6) with two molecular proportions of benzoylchloride in a known manner, or of bis-(3-acetylaminobenzene-1-sulfonyl-3'-aminobenzene-1'-sulfonyl)-benzidine-m-m'-disulfonic acid:



obtainable by acetylating the sodium salt of bis-(3-aminobenzene-1-sulfonyl-3'-aminobenzene-1'-sulfonyl)-benzidine-m-m'-disulfonic acid

also mixtures of the same among themselves or with other synthetic or vegetable tanning agents.

We claim:

1. A tanning composition, the active constituent of which is a condensation product of the probable formula:



wherein R stands for a benzene, naphthalene or diphenyl radical, both nuclei of the diphenyl radical being linked together directly or by means of a bridge, and R1 and R2 represent di- or polynuclear aryl-sulfone-arylamide derivatives of the benzene or naphthalene series with chain-like linkage in which the sulfone-imide groups combining the aryl nuclei may be partly replaced by aliphatic or aromatic carboxylic acid amide groups, and wherein at least one nucleus contains a sulfonic acid group, and wherein all nuclei may be further substituted by halogen or alkyl- or hydroxy- or carboxylic- or alkylacetylamino groups.

2. A tanning composition, the active constituent of which is a condensation product of the probable formula:



being a colorless powder easily soluble in water. 130

JOHANN HUISMANN.  
GUSTAV MAUTHE.

135

140

145

150

55 (British Letters Patent 333,559, Example 7) in an aqueous solution with an excess of acetic anhydride at a temperature of 40° C. in the presence of chalk and many other compounds of the like constitution. All these products are distinguished 60 by their strong tanning properties as, accordingly,

65

70

75